

## 1

3,009,767

**SEPARATION OF TRANSURANIC ELEMENTS  
FROM RARE EARTH COMPOUNDS**

Truman P. Kohman, Chicago, Ill., assignor to the United States of America as represented by the United States Atomic Energy Commission  
No Drawing. Filed Sept. 24, 1945, Ser. No. 618,408  
17 Claims. (Cl. 23—14.5)

The present invention relates to a process for the separation of certain transuranic elements from 4f-type rare earth and alkaline earth compounds and other impurities. More particularly, it is concerned with the separation of neptunium and plutonium from rare earth fission products and other impurities present in carrier precipitates by subjecting the latter to extraction with a solution in which the neptunium and plutonium compounds present in said precipitates are soluble, but in which the rare earth and alkaline earth compounds are insoluble, or substantially so.

It is known that plutonium can be produced in small quantities by the bombardment of uranium metal with slow or thermal neutrons. The designation "plutonium" or "element 94" as used throughout the present description refers to the transuranic element having an atomic number of 94. The expression "94<sup>239</sup>" means the isotope of element 94 has an atomic weight or mass of 239. Similarly, the terms "element 93" or "Np" refer to the new element known as neptunium having an atomic number of 93.

Uranium is composed of three isotopes, namely, U<sup>234</sup>, U<sup>235</sup> and U<sup>238</sup>, the latter being present in excess of 99 percent of the whole. When U<sup>238</sup> is subjected to the action of slow or thermal neutrons, a fourth isotope, U<sup>239</sup>, is produced having a half-life of 23 minutes and undergoes beta decay to Np<sup>239</sup> which decays further by beta radiation with a half-life of 2.3 days to yield plutonium. In addition to the formation of the transuranic elements, neptunium and plutonium, there are simultaneously produced other elements of lower atomic weight known as fission fragments. These fission fragments are composed of two distinct element groups, i.e., a light and heavy element group. The light group contains elements having atomic numbers of between about 35 and 46 while the heavier group is composed of elements of atomic numbers varying between about 51 and 60. The elements of these groups as originally produced are considerably overmassed and under charged and hence are highly unstable. By beta radiation, however, they quickly transform themselves into isotopes of these various elements having longer half-lives. The fission fragments and their resulting decay products are commonly known as fission products.

The various radioactive fission products have half-lives ranging from a fraction of a second to thousands of years. Those having very short half-lives may be largely eliminated by aging the material for a reasonable period before handling. Those with very long half-lives do not have sufficiently intense radiation to endanger personnel by moderate shielding. On the other hand, the fission products having half-lives ranging from a few days to a few years have dangerously intense radiations which cannot be eliminated by ageing for practical storage periods. These products are chiefly radioactive isotopes of

## 2

Sr, Y, Zr, Cb, and Ru of the light group and Te, I, Cs, Ba, La, Ce, and Pr of the heavy group.

It may be readily seen that plutonium produced as generally set forth above is contaminated with considerable quantities of uranium and fission products. In fact, the plutonium constitutes only a very minor portion of the irradiated mass i.e., rarely more than about one percent thereof by weight and not infrequently as low as one or several parts per million. In view of such a low concentration of plutonium in the irradiated metal, it becomes apparent that the procedure employed to recover that element must be highly efficient in order to be at all practicable.

There have been devised a number of procedures for the removal and concentration of plutonium from extremely dilute solutions thereof. In general, such methods involve the formation of various insoluble compounds in said dilute solutions in which the compounds are capable of carrying plutonium in a lower valent state not greater than 4, usually 3 or 4. The carrier precipitate and plutonium thus obtained are then dissolved and the plutonium oxidized to a valent state greater than 4, usually the hexavalent state, in which state of oxidation it is soluble in the presence of said carrier. Under these conditions, the plutonium remains in solution and the fission products are removed when the carrier compound is precipitated. Thereafter, the dissolved plutonium is reduced to a valence state in which it is carriable by the aforesaid or other carrier and removed from solution in the form of a carrier precipitate which may again be dissolved and the plutonium purified further if considered necessary or desirable by repeating the above cycle. This procedure obviously is cumbersome and time consuming since it requires a number of such steps in order to effect a substantial removal of fission products and other impurities.

It is an object of the present invention to provide a process by which plutonium and neptunium can be more efficiently separated from impurities such as, the rare earth and alkaline earth fission products normally associated therewith than has been afforded by prior methods.

A further object is to provide a process whereby it is possible to separate plutonium and neptunium from said rare earth and alkaline earth fission products without the utilization of involved oxidation-reduction steps formerly required to effect such separations.

A still further object is to provide a new process for the separation of the aforesaid transuranic elements from solutions containing uranium fission products, which involves first the simultaneous utilization of separate carriers for said transuranic elements and for fission products and thereafter employing a solvent which is capable of selectively extracting the transuranic elements and carrier therefor, leaving behind the fission products and carrier therefor in the form of a substantially insoluble residue.

Further objects will be apparent from the present description.

It has now been discovered that when carriers containing plutonium and neptunium, such as the tetrafluorides and dioxalates of thorium and uranium (+4 valence), are extracted at elevated temperatures with a solution of ammonium fluoride, ammonium oxalate, or a mixture thereof, the rare earth fission products as well as other im-

purities present therein may be readily separated from the neptunium and plutonium since the aforesaid rare earths and impurities are substantially insoluble in said solution whereas plutonium and neptunium as well as carriers of the above mentioned class are easily soluble therein. Otherwise expressed, the process of my invention may be specifically represented in substance as follows:



In accordance with a preferred embodiment of my invention, hydrogen fluoride is added to an acid solution of neutron irradiated uranium which has previously been subjected to the action of a suitable reducing agent such as, for example, sulphur dioxide, sodium nitrite, or ferrous ammonium sulphate in order to completely reduce the neptunium and plutonium present to the +4 or carriable state. In addition to the aforesaid components, such a solution likewise contains rare earth and alkaline earth fission products, a fission product carrier, and thorium or uranous ions depending on the particular plutonium carrier which it is desired to employ. On addition of the hydrogen fluoride, a precipitate of thorium fluoride, or uranium tetrafluoride is formed carrying with it the fluorides of plutonium and neptunium together with the insoluble fluorides of the rare earth fission products and their carrier. The precipitate thus formed is then separated by filtration or other convenient means after which it is extracted with an aqueous solution of ammonium fluoride, ammonium oxalate, or a mixture thereof at elevated temperatures such as, for example, from about 70 to 100° C., preferably at about 80 to 90° C., thereby extracting the thorium or uranium carrier component neptunium, plutonium, and a small quantity of rare earth fission products and carrier from said precipitate leaving behind as a substantially insoluble residue the fluorides of the rare earths and carrier therefor. To the solution thus formed is added a suitable mineral acid such as, for example, nitric acid to precipitate plutonium, neptunium, thorium fluoride, or uranium tetrafluoride and a greatly reduced quantity of rare earth fission products and carrier. In this connection the normality of the solution from which the plutonium and neptunium are precipitated may vary between the range, 0.01 to 10 N. In general, however, it has been found preferable to employ acidity ranges of between about 0.1 and 1.0 N.

Further separation of the neptunium, plutonium, and thorium, or uranium from rare earth fission products and carrier can be readily accomplished by repeating the above cycle. After the rare earths have thus been removed, the thorium fluoride, or uranium tetrafluoride carrier can be separated from the neptunium and plutonium by means of any of several suitable methods. It is preferred, however, to accomplish this object by metathesizing said carrier with strong alkali which involves reacting the carrier precipitate with an alkali metal hydroxide such as, for example, potassium or sodium hydroxides, to yield thorium or uranous hydroxides, either of which is readily soluble in nitric acid. The carrier precipitate which is converted by this treatment to the hydroxide is then washed with water to remove any fluoride ions which might be present after which it is dissolved in a suitable oxidizing medium such as, for example, one consisting of a mixture of nitric acid and potassium dichromate whereby the valence of the neptunium and plutonium contained therein is changed to the +6 state.

In the event thorium has been used as a carrier, the plutonium and neptunium may be precipitated by adding sodium acetate to the solution to form sodium plutonyl acetate and sodium neptunium acetate which are relatively insoluble compounds, leaving thorium in solution.

If uranium tetrafluoride is employed as a carrier, the solution which has been subjected to the oxidizing action of the nitric acid-potassium dichromate mixture contains neptunium, plutonium, and uranium in the hexavalent state and hence separation of the latter cannot be effected until the neptunium and plutonium have been selectively reduced to the +4 valence state. This can be accomplished by introducing into the solution a suitable reducing agent such as, for example, sodium nitrite or sulphur dioxide whereby the valence of neptunium and plutonium is changed from +6 to +4 while uranium is unaffected. The plutonium and neptunium can then be removed from solution by the formation of the iodate or peroxide in a known manner.

When the oxalates of thorium or uranium are employed as carriers for plutonium in the process of my invention, procedures slightly different from those set forth above should be utilized in separating said carriers from the neptunium and plutonium. Thus, after the rare earth fission products and other impurities have been removed, the carrier precipitate which consists of thorium, or uranium oxalates, neptunium, and plutonium is dissolved in a mixture of nitric acid and potassium dichromate. In the case of thorium carrier precipitates, the plutonium and neptunium present therein are oxidized to the +6 state and as such may be separated from thorium by the addition of sodium acetate to form insoluble sodium plutonyl acetate and sodium neptunyl acetate. As an alternate method, the thorium can be removed from solution by the addition of a suitable source of fluoride or oxalate ions. With uranium carrier precipitates, the whole is dissolved in a mixture of dichromate and nitric acid to oxidize the uranium, plutonium and neptunium to a valence of +6. To the resulting solution is then added a suitable reducing agent such as, for example, sodium nitrite, ferrous ammonium sulphate, or sulphur dioxide whereby the plutonium and neptunium present therein are reduced to the +4 valence state. Under these conditions plutonium and neptunium can readily be removed from the solution in the form of their iodates or peroxides in a known manner leaving the uranium in solution.

The quantity of fission product carrier utilized should not, in general, exceed a concentration greater than approximately ten times the amount of plutonium or plutonium carrier present. In the majority of instances, however, it is preferable to employ said fission product carrier in an amount substantially equivalent to the concentration of thorium or uranium carriers utilized. If ratios of fission product carrier to plutonium, or plutonium carrier greater than ten to one are used, it will be observed that it becomes very difficult to remove the plutonium from the fission product carrier precipitate owing to the fact that the plutonium is substantially enveloped by the fission product carrier, and thereby prevents satisfactory extraction of the plutonium by the solution of ammonium fluoride or ammonium oxalate. As examples of suitable rare earth and alkaline earth fission product carriers, there may be mentioned the fluorides and oxalates of lanthanum, cerium (+3 valence), strontium, calcium, yttrium and the like. Other compounds of fission product elements which are insoluble in the ammonium oxalate or fluoride solution and insoluble in the initial plutonium solution from which the plutonium is carried, also may be used.

In regard to the strength of the ammonium fluoride or ammonium oxalate solutions utilized in carrying out the process of my invention, it may generally be said that these two salts or a mixture thereof should preferably be present in quantities sufficient to provide a saturated solution at about 25° C., and it is to be strictly understood that the expression "aqueous saturated solution" appearing in certain of the appended claims is to be construed as a saturated solution of either of the aforesaid salts or a mixture thereof at the above indicated temperature.

The word "carrier," as generally considered, may be

regarded as a substantially insoluble solid, finely divided compound having an inorganic cation and containing an anion which is capable of forming a substantially insoluble compound with the particular cation it is desired to remove from solution. The word "carrier" as used herein with reference to the rare earth fission products is intended to mean a suitable lanthanum, strontium, cerous, or similar compound, whose anion is capable of forming a substantially insoluble compound with said rare earths.

In instances where plutonium and neptunium are present in macro amounts, i.e., about 50 mg. per liter and above, it is unnecessary to employ a carrier therefor since these elements will precipitate satisfactorily together with the rare earth fission products when hydrogen fluoride, oxalic acid or other suitable acid is added thereto. The precipitate thus formed can then be extracted with an aqueous solution of ammonium fluoride or ammonium oxalate in accordance with the procedure outlined above to effect a direct separation of neptunium and plutonium from the rare earth fission products and other impurities.

Where relatively large concentrations of neptunium are present and it is desirable to separate the same from plutonium, this object may be readily accomplished by selectively oxidizing the neptunium to the +6 or non-carriable state by the action of a mixture of sodium bromate and nitric and/or sulphuric acids at a temperature of about 50 to 70° C. for a period not to substantially exceed ten to fifteen minutes. Under such conditions the plutonium remains in the +4 or carriable state, and can be removed from the solution by merely adding hydrogen fluoride or oxalic acid provided the plutonium is present in macro quantities; if not, it can be satisfactorily separated by means of a suitable carrier such as, for example, thorium fluoride.

The present invention may be further illustrated by the following specific examples:

*Example 1*

Sufficient neutron irradiated uranium was dissolved in a liter of 1 M nitric acid to form a 21 percent solution of uranyl nitrate. To this solution was then added 3.5 grams of  $\text{Th}^{+4}$  ion as thorium nitrate, 1 gram of  $\text{Ce}^{+3}$  ion as cerium nitrate, 2.8 grams of ferrous ammonium sulphate, and 7.7 grams of hydrated oxalic acid ((COOH). $2\text{H}_2\text{O}$ ). The resulting mixture was agitated at 50° C. for two hours and then cooled to about 25° C. and agitated for an additional two hours after which the precipitate thus formed, containing plutonium and rare earth fission products, was separated by filtration. The residue thus obtained was washed with 30 milliliters of a solution, 0.015 M in oxalic acid and 1 M in nitric acid. The washed precipitate was next dissolved in 950 milliliters of 0.3 M ammonium oxalate, and the resulting solution heated with agitation for about one hour at 75 to 85° C. The hot solution was then filtered to remove the rare earth and other insoluble oxalates present after which 3.05 liters of 5 N nitric acid was added to the filtrate. The acidified solution was next heated at 75° C. for one hour in the presence of agitation, and then cooled to 25° C. and stirred for one hour. During this treatment a precipitate formed consisting essentially of plutonium, some neptunium, thorium oxalate, and a greatly reduced quantity of rare earth fission products and other impurities. Specifically, it was found that 99 percent of the rare earth fission products, 99.7 percent of the alkaline earths, and 75 percent of the zirconium present had been removed from the original precipitate in one cycle.

*Example 2*

To 4 milliliters of a solution containing 0.3 mg. of  $\text{Th}^{+4}$  as thorium nitrate, 0.3 mg. of  $\text{La}^{+3}$  as lanthanum nitrate, 600 counts/minute of plutonium<sup>+4</sup>, and 6,000 counts/minute of neptunium<sup>+4</sup>, was added sufficient hydrofluoric acid to render the resulting solution approximately 6 N after which the precipitated fluorides were centrifuged, and the supernatant liquor decanted. The

residue was next washed with 1 milliliter of water, centrifuged, the supernatant layer decanted, and the washed precipitate extracted with 5 milliliters of 10 N ammonium fluoride for 1 hour at 80° C. while agitating. The mixture was then cooled, centrifuged and 5 milliliters of nitric acid added to the supernatant liquor. As a result, a precipitate of thorium fluoride was formed which carried with it about 92 percent of the plutonium and approximately 93 percent of the neptunium originally present. Also, approximately 95 percent of the lanthanum percent in the original precipitate was removed in one cycle.

*Example 3*

The procedure and conditions employed were identical in all respects with those utilized in Example 1 except for the fact that the solution used to extract the thorium oxalate precipitate consisted of 950 milliliters of 5 N ammonium fluoride to which had been added sufficient ammonium oxalate to produce a saturated solution at 25° C. The quantity of rare earth fission products and alkaline earths removed from the thorium oxalate precipitate in one cycle amounted to 96 and 98 percent respectively.

While the examples given above are illustrative of certain specific applications of my invention, it should be particularly understood that I do not desire to be limited thereto since it will be apparent to those skilled in the art that said invention is susceptible of numerous modifications without departing from the scope thereof. In general, it may be said that any process involving the utilization of ammonium salt solutions of the aforesaid type to separate plutonium and/or neptunium from rare earth compounds is to be regarded as lying within the scope of my invention.

What is claimed is:

1. A process for the separation of transuranic values selected from the group consisting of plutonium and neptunium values from 4f-type rare earth and alkaline earth values which comprises extracting at elevated temperatures a solid composition containing said transuranic values, a carrier for said transuranic values selected from the group consisting of the oxalates and fluorides of thorium and uranium (+4 valence) and an impurity of the group consisting of rare earth and alkaline earth values and a carrier therefor selected from the group consisting of lanthanum fluoride, cerium trifluoride, strontium fluoride, calcium fluoride, yttrium fluoride, lanthanum oxalate, cerous oxalate, strontium oxalate and yttrium oxalate, with a solution of an ammonium salt selected from the group consisting of ammonium fluoride and ammonium oxalate, removing the insoluble matter which consists essentially of rare earth and alkaline earth values and carrier therefor, adding a mineral acid to the resulting solution to precipitate said transuranic values and the carrier for these transuranic values together with a greatly decreased concentration of rare earth and alkaline earth values, and repeating the above cycle to effect further separation of the transuranic values and carrier therefor from said rare earth and alkaline earth values.
2. A process for the separation of transuranic values selected from the group consisting of plutonium and neptunium values from 4f-type rare earth and alkaline earth values, which comprises extracting at elevated temperatures a solid composition containing essentially said transuranic values, a carrier for said transuranic values selected from the group consisting of the oxalates and fluorides of thorium and uranium (+4 valence), and rare earth and alkaline earth values and a carrier therefor selected from the group consisting of lanthanum fluoride, cerium trifluoride, strontium fluoride, calcium fluoride, yttrium fluoride, lanthanum oxalate, cerous oxalate, strontium oxalate, calcium oxalate and yttrium oxalate with a saturated solution of an ammonium salt selected from

the group consisting of ammonium fluoride and ammonium oxalate, removing the insoluble matter which consists essentially of rare earth and alkaline earth values and carrier therefor, adding nitric acid to the resulting solution to precipitate said transuranic values and the carrier for these transuranic values together with a greatly decreased concentration of rare earth and alkaline earth values, and repeating the above cycle to effect further separation of said transuranic values and carrier therefor from said rare earth and alkaline earth values.

3. A process for the separation of transuranic values selected from the group consisting of plutonium and neptunium values from 4f-type rare earth and alkaline earth values which comprises extracting at temperatures of between about 70 and 100° C. a solid composition containing essentially said transuranic values a carrier for said transuranic values selected from the group consisting of the oxalates and fluorides of thorium and uranium (+4 valence, and rare earth and alkaline earth values, and a carrier therefor selected from the group consisting of lanthanum fluoride, cerium trifluoride, strontium fluoride, calcium fluoride, yttrium fluoride, lanthanum oxalate, cerous oxalate, strontium oxalate, calcium oxalate and yttrium oxalate with a solution of an ammonium salt selected from the group consisting of ammonium fluoride and ammonium oxalate, removing the insoluble matter which consists essentially of rare earth and alkaline earth values and carrier therefor, adding nitric acid to the resulting solution to precipitate said transuranic values and the carrier for these transuranic values together with a greatly decreased concentration of rare earth and alkaline earth values, and repeating the above cycle to effect further separation of said transuranic values, and carrier therefor from said rare earth and alkaline earth values.

4. A process for the separation of transuranic values selected from the group consisting of plutonium and neptunium values from 4f-type rare earth and alkaline earth values which comprises extracting at temperatures of between about 80 and 90° C. a solid composition containing essentially said transuranic values a carrier for said transuranic values selected from the group consisting of the oxalates and fluorides of thorium and uranium (+4 valence, and rare earth and alkaline earth values, and a carrier therefor selected from the group consisting of lanthanum fluoride, cerium trifluoride, strontium fluoride, calcium fluoride, yttrium fluoride, lanthanum oxalate, cerous oxalate, strontium oxalate, calcium oxalate and yttrium oxalate with a solution of an ammonium salt selected from the group consisting of ammonium fluoride and ammonium oxalate, removing the insoluble matter which consists essentially of rare earth and alkaline earth values and carrier therefor, adding nitric acid to the resulting solution to precipitate said transuranic values and the carrier for these transuranic values together with a greatly decreased concentration of rare earth and alkaline earth values, and repeating the above cycle to effect further separation of said transuranic values, and carrier therefor from said rare earth and alkaline earth values.

5. A process for the separation of transuranic values selected from the group consisting of plutonium and neptunium values from 4f-type rare earth and alkaline earth values, which comprises extracting at a temperature of between about 70 and 100° C. a solid composition containing essentially transuranic values, a carrier for said transuranic values selected from the group consisting of the oxalates and fluorides of thorium and uranium (+4 valence), and rare earth and alkaline earth values, and a lanthanum carrier therefor with a saturated aqueous solution of an ammonium salt selected from the group consisting of ammonium fluoride and ammonium oxalate, removing the insoluble matter which consists essentially of rare earth and alkaline earth values and carrier therefor, adding a mineral acid to the resulting solution to precipitate said transuranic values and the carrier for these transuranic values together with a greatly decreased concen-

tration of rare earth and alkaline earth values, and repeating the above cycle to effect further separation of said transuranic values and carrier therefor from said rare earth and alkaline earth values.

6. A process for the separation of transuranic values selected from the group consisting of plutonium and neptunium values from 4f-type rare earth and alkaline earth values, which comprises extracting at temperatures of between about 80 and 90° C. a solid composition containing essentially said transuranic values, a thorium oxalate carrier for said transuranic values, and rare earth and alkaline earth values and a cerium (+3 valence) carrier therefor with an aqueous saturated solution of ammonium oxalate, removing the insoluble matter which consists essentially of rare earth and alkaline earth values and the cerium carrier therefor, adding nitric acid to the resulting solution to precipitate said transuranic values and the thorium oxalate carrier for these transuranic values together with a greatly decreased concentration of rare earth and alkaline earth values, and repeating the above cycle to effect further separation of said transuranic values and thorium oxalate from said rare earth and alkaline earth values.

7. A process for the separation of transuranic values selected from the group consisting of plutonium and neptunium values from 4f-type rare earth and alkaline earth values, which comprises extracting at temperatures of between about 80 and 90° C. a solid composition containing essentially said transuranic values, a thorium fluoride carrier for said transuranic elements, and rare earth and alkaline earth values, and a lanthanum carrier therefor with an aqueous saturated solution of ammonium fluoride, removing the insoluble matter which consists essentially of rare earth and alkaline earth values and the lanthanum carrier therefor, adding nitric acid to the resulting solution to precipitate said transuranic values and the thorium fluoride carrier for these transuranic values together with a greatly decreased concentration of rare earth and alkaline earth values, and repeating the above cycle to effect further separation of said transuranic values and thorium fluoride from said rare earth and alkaline earth values.

8. A process for the separation of transuranic values selected from the group consisting of plutonium and neptunium values from 4f-type rare earth and alkaline earth values, which comprises extracting at a temperature of between about 70 and 100° C. a solid composition containing essentially said transuranic values, a thorium oxalate carrier for said transuranic elements, and rare earth and alkaline earth values and cerium (+3 valence) carrier therefor with a saturated aqueous solution of a mixture of ammonium fluoride and ammonium oxalate, removing the insoluble matter which consists essentially of rare earth and alkaline earth values and cerium carrier therefor, adding nitric acid to the resulting solution to precipitate said transuranic values and thorium oxalate together with a greatly decreased concentration of rare earth and alkaline earth values, and repeating the above cycle to effect further separation of said transuranic values and thorium oxalate from said rare earth and alkaline earth values.

9. A process for the separation of transuranic values selected from the group consisting of plutonium and neptunium values from 4f-type rare earth and alkaline earth values, which comprises extracting at temperatures of between about 70 and 100° C. a solid composition containing essentially said transuranic values, a carrier for said transuranic values selected from the group consisting of oxalates and fluorides of thorium and uranium (+4 valence), and rare earth and alkaline earth values and a carrier therefor selected from the group consisting of lanthanum fluoride, cerium trifluoride, strontium fluoride, calcium fluoride, yttrium fluoride, lanthanum oxalate, cerous oxalate, strontium oxalate, calcium oxalate and yttrium oxalate, with a solution of ammonium salt

selected from the group consisting of ammonium fluoride and ammonium oxalate, removing the insoluble matter which consists essentially of rare earth and alkaline earth values and carrier therefor, adding thereto sufficient mineral acid to produce a solution whose acidity ranges between 0.01 and about 10.0 N thereby resulting in the precipitation of said transuranic values and the carrier for these transuranic values together with a greatly decreased concentration of rare earth and alkaline earth values, and repeating the above cycle to effect further separation of said transuranic values and carrier therefor from said rare earth and alkaline earth values.

10. A process for the separation of transuranic values selected from the group consisting of plutonium and neptunium values from 4f-type rare earth and alkaline earth values, which comprises extracting at temperatures of between about 70 and 100° C. a solid composition containing essentially said transuranic values, a carrier for said transuranic values selected from the group consisting of oxalates and fluorides of thorium and uranium (+4 valence), and rare earth and alkaline earth values and a carrier therefor selected from the group consisting of lanthanum fluoride, cerium trifluoride, strontium fluoride, calcium fluoride, yttrium fluoride, lanthanum oxalate, cerous oxalate, strontium oxalate, calcium oxalate and yttrium oxalate, with a solution of ammonium salt selected from the group consisting of ammonium fluoride and ammonium oxalate, removing the insoluble matter which consists essentially of rare earth and alkaline earth values and carrier therefor, adding thereto sufficient mineral acid to produce a solution whose acidity ranges between 0.1 and about 1.0 N, thereby resulting in the precipitation of said transuranic values and the carrier for these transuranic values together with a greatly decreased concentration of rare earth and alkaline earth values, and repeating the above cycle to effect further separation of transuranic values and carrier therefor from said rare earth and alkaline earth values.

11. In a process for the separation of transuranic values selected from the group consisting of plutonium and neptunium values from 4f-type rare earth and alkaline earth fission product values, the steps which comprise contacting a solution containing said transuranic values in a valence state not greater than 4 and rare earth and alkaline earth fission values with a carrier for said fission products selected from the group consisting of lanthanum fluoride, cerium trifluoride, strontium fluoride, calcium fluoride, yttrium fluoride, lanthanum oxalate, cerous oxalate, strontium oxalate, calcium oxalate and yttrium oxalate and a carrier for said transuranic values selected from the group consisting of the oxalates and fluorides of thorium and uranium (+4 valence), recovering the precipitate thus obtained and extracting it with a selective solvent for said transuranic values and carrier therefor comprising a solution of an ammonium salt selected from the group consisting of ammonium fluoride and ammonium oxalate, and removing from the resulting solution the insoluble matter present therein which consists essentially of rare earth and alkaline earth values and carrier therefor.

12. In a process for the separation of transuranic values selected from the group consisting of plutonium and neptunium values from uranium fission products the steps which comprise contacting the solution containing said transuranic values in a valence state not greater than 4 and said fission products with a carrier for said transuranic values selected from the group consisting of the oxalates and fluorides of thorium and uranium (+4 valence) and a lanthanum carrier for said fission products, recovering the precipitate thus obtained and extracting it with a selective solvent for said transuranic values and carrier therefor comprising a solution of an ammonium salt selected from the group consisting of ammonium fluoride and ammonium oxalate, and removing from the resulting solution the insoluble matter present therein

which consists essentially of uranium fission products and carrier therefor.

13. In a process for the separation of transuranic values selected from the group consisting of plutonium and neptunium values from uranium fission products, the steps which comprise contacting a solution containing said transuranic values in a valence state not greater than 4 and uranium fission products with a carrier for said transuranic values comprising thorium oxalate and a carrier for said fission products comprising cerous oxalate, recovering the precipitate thus obtained and extracting it at a temperature of between about 80 and about 90° C. with an aqueous saturated solution of ammonium oxalate, and removing from the resulting solution the insoluble matter present therein which consists essentially of uranium fission products and cerous oxalate.

14. In a process for the separation of transuranic values selected from the group consisting of plutonium and neptunium values from uranium fission products, the steps which comprise contacting a solution containing said transuranic values in a valence state not greater than 4 and uranium fission products with a carrier for said transuranic values comprising thorium fluoride and a carrier for said fission products comprising lanthanum fluoride, recovering the precipitate thus obtained and extracting it at a temperature of between about 80 and about 90° C. with an aqueous saturated solution of ammonium fluoride, and removing from the resulting solution the insoluble matter present therein which consists essentially of uranium fission products and lanthanum fluoride.

15. A process for the separation of transuranic values selected from the group consisting of plutonium and neptunium values from 4f-type rare earth and alkaline earth values which comprises extracting at elevated temperatures a solid composition containing said transuranic values, a carrier for said transuranic values selected from the group consisting of the oxalates and fluorides of thorium and uranium (+4 valence), and an impurity of the group consisting of rare earth and alkaline earth values and a carrier therefor selected from the group consisting of lanthanum fluoride, cerium trifluoride, strontium fluoride, calcium fluoride, yttrium fluoride, lanthanum oxalate, cerous oxalate, strontium oxalate, calcium oxalate and yttrium oxalate with a solution of an ammonium salt selected from the group consisting of ammonium fluoride and ammonium oxalate.

16. A process for the separation of neptunium values from 4f-type rare earth and alkaline earth values which comprises extracting at elevated temperatures a solid composition containing said neptunium values, a carrier for said neptunium values selected from the group consisting of the oxalates and fluorides of thorium and uranium (+4 valence), an impurity of the group consisting of rare earth and alkaline earth values and a carrier therefor selected from the group consisting of lanthanum fluoride, cerium trifluoride, strontium fluoride, calcium fluoride, yttrium fluoride, lanthanum oxalate, cerous oxalate, strontium oxalate, calcium oxalate and yttrium oxalate with a solution of an ammonium salt selected from the group consisting of ammonium fluoride and ammonium oxalate, removing the insoluble matter which consists essentially of rare earth and alkaline earth values and carrier therefor, adding a mineral acid to the resulting solution to precipitate said neptunium values and the carrier therefor together with a greatly decreased concentration of rare earth and alkaline earth values, and repeating the above cycle to effect further separation of neptunium values and carrier therefor from said rare earth and alkaline earth values.

17. A process for the separation of plutonium values from 4f-type rare earth and alkaline earth values which comprises extracting at elevated temperatures a solid composition containing said plutonium values, a carrier for said plutonium values selected from the group consist-

ing of the oxalates and fluorides of thorium and uranium (+4 valence), an impurity of the group consisting of rare earth and alkaline earth values and a carrier therefor selected from the group consisting of lanthanum fluoride, cerium trifluoride, strontium fluoride, calcium fluoride, yttrium fluoride, lanthanum oxalate, cerous oxalate, strontium oxalate, calcium oxalate and yttrium oxalate with a solution of an ammonium salt selected from the group consisting of ammonium fluoride and ammonium oxalate, removing the insoluble matter which consists

5

10

essentially of rare earth and alkaline earth values and carrier therefor, adding a mineral acid to the resulting solution to precipitate said plutonium values and the carrier therefor together with a greatly decreased concentration of rare earth and alkaline earth values, and repeating the above cycle to effect further separation of plutonium values and carrier therefor from said rare earth and alkaline earth values.

No references cited.